# EUROPEAN PATENT APPLICATION

(11) **EP 4 663 862 A1**
(43) Date of publication of application: **17.12.2025**
(21) Application number: 24204489.9
(22) Date of filing: 03.10.2024
(51) Int. Cl.: E04B 1/12, E04C 5/07

(54) **A CONSTRUCTION REINFORCEMENT, A CONSTRUCTION ELEMENT COMPRISING THE CONSTRUCTION REINFORCEMENT, A METHOD FOR OBTAINING THE CONSTRUCTION ELEMENT, AND USE OF THE CONSTRUCTION ELEMENT**

(30) Priority: 14.06.2024 EP 24461587
(71) Applicant: Innowacje Michal Halas, 81-593 Gdynia (PL)
(72) Inventor: Halas, Michal, 81-593 Gdynia (PL); Jerzy, Obojski, Krakow (PL)
(74) Representative: AOMB Polska Sp. z.o.o.

(57) **Abstract**

A construction reinforcement suitable for use in concrete-based systems, comprising at least one board (101) made of Fiber Reinforced Polymers (FRP), characterized in that the board is made of retired FRP, and wherein the construction reinforcement comprises means for improving adhesion to concrete and the force transmission. A construction element comprising the construction reinforcement embedded in concrete. A method for obtaining the construction element.

## Description

### Technical Field

The present invention relates to the field of non-metallic construction reinforcements, named by inventor "Stolat", for use in construction applications. More specifically, the invention relates to boost performance of a concrete-based systems comprising construction reinforcements made of **retired** Fiber Reinforced Polymers (FRP).

### Prior Art

Fiber Reinforced Polymers (FRP) are advanced composite materials that find extensive applications across various fields of engineering, with a significant impact in the construction industry. The primary advantage of FRP lies in its exceptional tensile strength and resistance to corrosion, which makes it a highly attractive alternative to traditional reinforcing materials such as steel. Alternative composite materials, such as carbon, glass, basalt, flax or aramid fiber reinforced polymers, can also be used to reinforce concrete, offering the added benefits of higher strength and corrosion resistance. FRP composites are composed of a polymer matrix that is reinforced with fibres, which can be derived from diverse materials such as glass, carbon, basalt or aramid fibres. Due to these intrinsic properties, FRP materials are increasingly being utilized as reinforcement in concrete structures, particularly in scenarios where traditional steel reinforcement may be prone to corrosion, especially in aggressive or harsh environmental conditions.

The use of FRP as reinforcement offers a multitude of benefits that collectively contribute to the construction of longer-lasting structures with reduced maintenance costs. Firstly, FRP reinforcement exhibits high chemical resistance, making it ideally suited for applications in environments that are exposed to salts, acids, and other corrosive substances. This high level of chemical resistance ensures that structures reinforced with FRP maintain their integrity and performance over extended periods, even under harsh conditions. Additionally, FRP composites are lightweight, which significantly facilitates their transport and installation, thereby reducing labour costs and simplifying the construction process.

Moreover, due to their dielectric properties, FRP materials can be effectively used in applications where electrical insulation is required, thus broadening their scope of utility. The introduction of FRP as a reinforcement material in construction not only enhances the durability and resilience of engineering structures but also opens up new design and technological possibilities. This innovative use of FRP allows for the creation of structures that are not only more durable but also capable of withstanding the demanding conditions of modern construction environments. As a result, the adoption of FRP in construction represents a forward-looking approach that leverages cutting-edge material science to achieve superior performance and sustainability in building practices. FRPs can also be used in installations where protection against electromagnetic interference (EMI) and radio frequency interference (RFI) is required, expanding their range of applications in modern construction projects.

Document US20240084590A1 describes a consumable formwork that remains part of the final structure, providing sufficient tensile strength to reduce or eliminate the need for steel reinforcement. This formwork system, made from rigid plastic and/or fiberglass reinforced plastic, interacts with poured concrete to create durable ceilings and roofs, and can incorporate low carbon concrete to reduce emissions. The formwork is used in constructing residential or commercial buildings, specifically for creating arched ceilings, flat roofs, or flat floors.

Document US2021017766A1 describes an improved construction of fiber-reinforced plastic (FRP) rebar and methods of manufacturing it. The new design has increased tensile strength, modulus of elasticity, and durability compared to traditional FRP rebar. These rebars are produced through a pultrusion process using continuous glass fibers and vinyl ester resin, which ensures higher glass content and corrosion resistance.

Document IN3306MUM2012A describes an invention related to building construction, specifically focusing on the use of fiber-reinforced plastic (FRP) for rebar in concrete structures. This new type of rebar addresses the limitations of traditional steel rebar, such as corrosion, by being fully corrosion-proof and offering higher tensile strength and lower weight. The FRP rebar is easier to install and maintains structural integrity better over time, leading to more durable and cost-effective concrete constructions.

Document US6401286B1 describes form decking for bridge decks, which aids in the forming and pouring of concrete. The system uses interlocking plastic forms with male and female tabs, allowing them to lock together and providing a smooth finish when removed. The bottom of the form is designed with ribs for reinforcement and strength. The use of plastic makes the forms more durable and allows for repeated use, making the construction process quick, easy, and efficient.

**The present invention** represents a significant advancement in the field of construction materials by introducing a novel type of construction reinforcement made from retired Fiber Reinforced Polymers (FRP). Unlike traditional steel reinforcement, the upcycled FRP reinforcement offer superior performance characteristics, including enhanced durability and corrosion resistance, which make them particularly suitable for use in aggressive environmental conditions, such as marine or chemically hostile environments. The use of upcycled FRP not only contributes to environmental sustainability by reducing waste and lowering the carbon footprint but also provides a higher strength-to-weight ratio, which improves the overall efficiency and longevity of construction projects. This innovative reinforcement is cheaper than conventional FRP reinforcement and addresses key issues associated with retired FRP used as reinforcement, such as weak bonding with concrete and the risk of delamination under tensile stress, by employing techniques (mostly recesses and protrusions) to strengthen bonding with concrete and means of deeply installed fasteners or ropes or deep holes preserving structural integrity of the FRP. Additionally, the application of protective nanocomposite coatings and the potential use of alternative bonding techniques, such as ultrasonic welding, further enhance the performance and reliability of the reinforcement. By leveraging these unique features, the present invention surpasses traditional methods, offering a more resilient, cost-effective, and environmentally friendly solution for modern construction needs.

### Summary of the Invention

According to the invention a construction reinforcement suitable for use in concrete-based systems, comprising at least one board made of Fiber Reinforced Polymers (FRP), and wherein the board is made of retired FRP, and wherein the construction reinforcement comprises means for improving adhesion to concrete and the force transmission.

Preferably the means for improving adhesion to concrete and the force transmission are selected from the group comprising protruding elements, through holes, grooves, indentations, adhered loose materials and/or combination of them.

Preferably the protruding elements are selected from the group comprising screws, pegs, bolts, dowels, plugs, expansion anchors, fasteners made of retired FRP, strings, strands, knots, retired fishing nets, bottle cups, polymer tines, rebars, FRP chunks, convex elements, and/or combination thereof.

Preferably the adhered loose materials ale selected from the group comprising sand, polymer elements, FRP elements, ground FRP dust, epoxy resin, gravel, aggregates, quartz, broken glass, perlite, ceramic, corundum, polyurethane powder, pumice, silicon carbide, and/or combination thereof.

Preferably the through holes have dimensions in the range from 10 to 990 mm, wherein the drilling angle is in the range from 40 to 140 degrees.

Preferably the board is substantially flat or is profiled into a shape selected from a group comprising a comb, an angled board, a U-shaped board, a L-shaped board H-shaped T-shaped, and/or a circular board.

Preferably the boards are butt jointed or at least partially overlapping.

Preferably the butt joint is a straight joint, a diagonal joint, a structural diagonal joint, a multiple tongue and groove joint or a structural joint.

Preferably the boards are jointed by adhesive and/or by other means, selected from the group comprising dovetail, pegs, dowels, plugs, expansion anchors, bolts, nails, screws, nails and/or combination thereof.

Preferably the boards are arranged in at least two parallel planes connected by FRP brackets, wherein the axial distance of the planes is in the range from 20 mm to 990 mm.

Preferably the construction comprises an upper and a lower boards, two side boards and means for stabilizing the folded construction in a 90 degrees angle position, and means for allowing the construction to be folded and unfolded.

Preferably the means for stabilizing the folded construction are selected from the group comprising strings, triangular elements, squared sticks, bear claw screws, and/or combination of them and the means for allowing the construction to be folded and unfolded are selected from the group comprising hinges, plugs, nails, screws, wedges, elastic strings, comb elements, 3D printed elements, strings, ropes, boards, elements with snap-fits and/or combination thereof.

Another aspect is a construction element comprising the construction reinforcement embedded in concrete of the thickness in the range from 20 mm to 9900 mm, wherein the concrete comprises aggregates, water and cement, and wherein the cement is selected from the group comprising Portland cement, geopolimers, fly ashes, blast furnace slag, belite cement, cement from agricultural ashes, aluminous cement, pozzolanic cement, silica fume, polymer functioning as binder, metakaolin, and and/or any combination thereof.

Another aspect is a method for obtaining the construction element, comprising following steps:
a) placing in the board the means for improving adhesion to concrete and force transmission, selected from the group comprising: screws, pegs, bolts, dowels, plugs, expansion anchors, fasteners made of retired FRP, strings, strands, knots, retired fishing nets, bottle cups, polymer tines, rebars, FRP chunks, convex elements, grooves, indentations, adhered loose materials selected from the group comprising sand, polymer elements, FRP elements, ground FRP dust, epoxy resin, gravel, aggregates, quartz, broken glass, perlite, ceramic, corundum, polyurethane powder, pumice, silicon carbide, and/or combination thereof **AND/OR**
   drilling the through holes in the boards, in the distance not less than 10 mm from the edges of the board and from any other hole;
b) optionally, covering all uncoated cut edges of the board with polymer;
c) jointing of boards;
d) pouring the reinforcement construction obtained in steps a)-c) with concrete material with a thickness of at least 20 mm or dipping the reinforcement construction into fresh concrete material with a thickness of at least 40 mm;
e) optionally vibrating and curing the concrete at a time of at least 2 hours.

Preferably after step c) protruding elements on the joints between boards using adhesive and/or other means, selected from the group comprising nails, screws, pegs, bolts, dowels, plugs, expansion anchors, fasteners made of retired FRP, strings, strands, knots, retired fishing nets, bottle cups, polymer tines, rebars, FRP chunks, convex elements, and/or combination thereof are installed.

Preferably the polymer is selected from the group comprising gelcoat, epoxy resin, polyurethane coatings, phenolic coatings, urea-formaldehyde coatings, polyester coatings, vinyl ester resins, silicone coatings, acrylic coatings, alkyd coatings, nitrocellulose coatings, melamine-alkyd coatings, nanocoatings and/or any combination thereof.

Preferably before pouring the concrete in step d) the reinforcement construction is prestressed by pulling a tensile force from 0,5 kN to 990 kN from both opposite ends of the construction.

Preferably the adhesive is selected from the group comprising polyurethane adhesives (PUR), epoxy adhesives, cyanoacrylate adhesives, acrylic adhesives, silicone adhesives, construction adhesives, contact adhesives, hybrid adhesives, cementitious adhesives, and/or parquet adhesives

Another aspect is a use of the construction element in the construction of roads and load-bearing structural elements like foundations, ceilings, footings, girders, columns, stairs, beams, retaining walls, concrete slabs, prefabricated concrete modules.

This invention addresses the need for sustainable construction materials by utilizing retired FRP, which not only contributes to environmental conservation but also offers superior mechanical properties compared to traditional metallic rebars. The upcycled reinforcement provide increased durability, resistance to corrosion, and improved strength-to-weight ratios, making them ideal for long-lasting and resilient construction projects at low cost. Furthermore, the innovation aims to optimize the bonding and compatibility of these reinforcements with various concrete mixtures, ensuring optimal load distribution and structural integrity in reinforced concrete structures. This makes the present invention particularly valuable for applications in harsh environments, such as marine or chemically aggressive settings, where conventional steel rebars would typically degrade.

The disclosed method addresses two key problems associated with retired FRP: the weak grip between concrete and FRP reinforcement and the delamination of FRP under high tensile stress. By cutting retired FRP into the largest possible pieces with minimal cutting, the method conserves effort and energy while enhancing the mechanical properties of the reinforced concrete. This approach improves the bond between FRP and concrete, reducing slippage, and maintains the structural integrity of FRP, minimizing the risk of delamination. Additionally, it ensures a more sustainable recycling process, reducing labor and energy costs, and ultimately leads to more durable and reliable reinforced concrete structures.

When concrete is reinforced with FRP, the bond between the two materials is crucial for effective load transfer and overall structural performance. Traditional FRP reinforcement methods often face challenges in ensuring a strong bond, primarily due to the smooth surface of FRP materials, which can lead to slippage and insufficient stress distribution. This weak grip can result in poor performance under load and reduce the overall durability of the structure.

Delamination is a critical issue for FRP materials, especially under high tensile stress. It occurs when the layers of FRP begin to separate, which can compromise the material's structural integrity and its ability to reinforce concrete effectively. Delamination can be exacerbated by the repeated cutting and handling of FRP, which can introduce defects and weak points.

By cutting the retired FRP into the largest possible pieces with minimal cutting, the method reduces the number of cuts and the associated risk of introducing defects that could lead to delamination. Larger FRP pieces retain their inherent structural integrity better than smaller, more frequently cut pieces. This helps maintain the FRP's tensile strength and resistance to delamination, ensuring that it can effectively contribute to the overall strength and durability of the reinforced concrete structure. Through pins, bolts and fastening elements are disclosed here to also help against delamination.

In addition to the mechanical benefits, the method is designed to be efficient in terms of effort and energy consumption. Traditional recycling processes for FRP often involve extensive cutting, crushing, reshaping, and sometimes chemical processing, which can be labor-intensive and energy-consuming. By opting to cut the FRP into the largest feasible pieces, the method conserves both effort and energy. This not only makes the recycling process more sustainable but also reduces the costs associated with labor and energy consumption.

The ecological benefits of using upcycled Fiber Reinforced Polymers (FRP) in construction are substantial and multifaceted. This innovative approach significantly reduces the environmental impact compared to traditional steel reinforcement methods. Firstly, the use of upcycled FRP drastically cuts down on waste, diverting large amounts of material from landfills and repurposing them into valuable construction resources. This contributes to a circular economy and promotes sustainable material management. Secondly, the production and processing of upcycled FRP require considerably less energy than the production of new steel reinforcement or new FRP reinforcement, leading to significant energy savings. Additionally, the use of upcycled FRP substantially lowers greenhouse gas emissions, including CO2, as it avoids the intensive energy and resource requirements associated with mining, refining, and manufacturing new steel. The result is a reduced carbon footprint, making the construction process more environmentally friendly. By integrating upcycled FRP into construction projects, the present invention not only enhances the sustainability of building practices but also provides a high-performance, durable alternative to traditional materials, aligning with global efforts to mitigate climate change and promote ecological stewardship.

The application of upcycled Fiber Reinforced Polymer (FRP) reinforcement in various construction environments highlights its versatility and superior performance. This innovative reinforcement has been extensively tested and proven to be exceptionally effective in harsh conditions, including marine and chemically aggressive environments. In marine applications, the upcycled FRP reinforcement demonstrates outstanding resistance to saltwater corrosion, making it ideal for constructing docks, piers, and underwater structures. Data from strength tests conducted in these environments show that the FRP reinforcement maintains its structural integrity and performance over extended periods, even when exposed to constant moisture and salt. Similarly, in chemically aggressive settings, such as industrial plants and wastewater treatment facilities, the upcycled FRP reinforcement exhibits high resistance to acidic and alkaline substances. Test results indicate that it outperforms traditional steel rebar, which often corrodes and deteriorates under such conditions. The advanced bonding techniques used in the production of FRP reinforcement ensure a strong adhesion with concrete and the force transmission, further enhancing its durability and load-bearing capacity. These specific use cases, supported by empirical data from rigorous testing, demonstrate that upcycled FRP reinforcement is not only a sustainable and environmentally friendly alternative but also a highly effective solution for reinforcing concrete in the most demanding construction environments.

If the word "concrete" is used, it refers to the conventional mixture commonly utilized in construction, which typically consists of sand, gravel, water, and Portland Cement. Additionally, advanced concrete materials such as self-healing concrete or ultra-high-performance concrete (UHPC) can be used in combination with the upcycled FRP reinforcement to enhance the overall structural performance and durability of the construction. This standard combination is widely recognized and employed due to its proven effectiveness and durability in a variety of construction applications. However, it is important to note that "concrete" in this context also encompasses variations that incorporate alternative materials to replace traditional components. For instance, polymer or fly ash may be used as a substitute for cement, and crushed glass can replace gravel, among other sustainable and innovative alternatives.

Furthermore, the term "concrete" should be understood to include geopolymer concrete and other advanced product like polymer concrete replacement products. Geopolymer concrete, for example, is made from industrial by-products and offers enhanced performance characteristics such as increased resistance to chemicals and lower carbon emissions compared to traditional Portland Cement-based concrete. These alternative concretes are increasingly being adopted in modern construction practices due to their environmental benefits and superior durability. Therefore, whenever "concrete" is mentioned, it should be interpreted broadly to cover not only the conventional mixture but also these innovative and sustainable alternatives that are designed to meet specific performance criteria and environmental standards in construction projects.

### Brief Description of the Drawings

In order to provide more complete understanding of the claimed invention and advantages thereof, the following description provides an explanation of possible exemplary embodiments thereof with a reference to figures of the appended drawings, wherein identical designations denote identical parts, and which illustrate the following:
Figs. 1a-1b show a construction reinforcement made of retired FRP boards (101), before pouring concrete or other curing material;
Figs. 2a-2b show the alternative way to connect the FRP boards (101);
Figs. 3a-f show the use of long pieces of polymer string and other added elements improving the connection between the concrete and the reinforcement; fig. 3g shows grooving for improving said connection; fig. 3h-i show the hybrid of retired FRP board and new steel or FRP rebars; fig.3j shows foldable reinforcement; fig. 3k shows reinforcement using biscuit joints; Fig. 3l-m show stirrups/ties made of retired FRP board; Fig.3n shows examples of H-shapes boards for better force transfer with concrete.
Fig. 4 shows a construction reinforcement where at least one board is not flat, but angled at one edge;
Fig. 5 shows a top view of nine retired FRP boards joined together with adhesive and nails and/or screws into large rectangular shape;
Figs. 6 a-c show a cross-sectional view of concrete block (a and b) and road (c) with two parallel planes of a construction reinforcements;
Fig. 7a shows an example of a making of reinforcement which is straight alternative to rebar;
Fig.7b shows setup for mass production of reinforcement similar to depicted at fig. 7a;
Fig. 8 shows an example of FRP board prepared for better grip with concrete by wavy cut;
Fig. 9 shows the use of bear claw screws improving connection between concrete and FRP reinforcement, this also counteracts delamination;
Figs. 10a-e show the procedure of joining two retired FRP boards (a) "side to side" for larger size reinforcement and (b-e) not warping joint of 2 retired FRP boards "face to face" glued for larger size reinforcement for concrete;
Figs. 11a-c show an example of retired FRP reinforcement specially for in factory concrete modules production and foldable reinforcement;
Fig. 12 discloses half of large circular foundation reinforcement, good for windmill generator;
Fig. 13a shows an example of a construction reinforcement build from comb elements (half-lap joint);
Figs. 13b-d show folding reinforcement to ease transportation;
Figs. 14 a-c show retired FRP reinforcements with holes, string (a) flat and (b-c) 3-dimensional;
Figs. 15 a-d show a cut out view of a bridge (or other supported horizontal construction element) beam/girder reinforcement made from retired FRP boards; Figs. 15 e-h disclose (e) making of I-beam and (f-g) examples of such I-beam as reinforcement with concrete; Fig. 15h shows untypical I-beam with curved bottom part; Fig. 15i shows beam/girder reinforcement made from retired FRP half circular element with simpler rooting in concrete than depicted at fig. 15d.
Figs. 16a-c show products from retired FRP which can work as alternative for dowel bar;
Figs. 17a-c show preparing a construction reinforcement using efficient cuts of retired windblade;
Figs. 18a-c show the procedure of making holes and convex elements for strengthening bond between FRP and concrete;
Fig. 19 shows a process of cutting of retired wind blade and other retired FRP elements.
Fig. 20a-g show folding reinforcements - easy to transport when flat.
Fig. 21 shows a cheap ground compression construction made of large retired FRP, concrete arc, tensioning cables and filtering fabric.

Main designations:
101 - FRP board;
102 - FRP fastening element;
103 - FRP protruding element;
104 - through hole;
105 - reinforcement prepared by butt joint of the boards 101;
106 - screw;
107 - trapezoidal fastening element and corresponding opening in the board 101;
108 - trapezoidal protruding peg and corresponding opening in the board 101;
109 - arrow indicating a direction of joining;
110 - through hole;
201 - joined reinforcement;
202 - glued joint;
301 - polymer string;
302 -fishing net;
303 - bottle cap;
304 - flat piece of PET bottle;
305 - flat piece of PET bottle cut in many tines;
306 - toothed rectangle;
307 - polymer tines;
308 - coarse sand;
309 - glossy epoxy area;
310 - rough area;
311 - brush;
312 - roller;
313 - string;
314-extrusion head;
315 - grooves;
316 - milling head;
317 - grooving;
318 - raised edges;
319 - grooving hook;
320 - rotating saw;
321 - press;
322 - rebar;
323 - rectangular hole;
324 - H-board with snap-fits;
325 - hole;
326 - stabilizing triangle;
327 - biscuit joint;
328 - incision;
329 - flexible clamp;
330 - zip tie (tie wrap);
331 -wire wheel brush;
332 - rasp;
333 - sandpaper;
334 - semicircular groove;
401 - contact area;
501 - element to pull the large module 502;
502 - module of multiple joint boards 101;
503 - module of multiple joint boards 101;
504 - fastener of different shapes;
505 - rope;
506 - element to pull the large module 502
601 - FRP bracket;
602 - concrete;
603 - top layer;
604 - screw;
701 - indentation;
702 - FRP chunk;
703 - groove;
704 - FRP board;
705 - duct system;
706 - rotating saw;
707-thread cutter;
708 - battery of sprinklers;
709 - battery of saw dust heads;
801 - narrow band saw;
802 - wavy edges;
803 - planned wavy path to be cut;
901 - narrow hole;
902 - bear claw screw;
903 - bear claw screw;
1001 - screw/bolt/nail;
1002 - screw/bolt/nail;
1003 - screw/bolt/nail;
1004 - peg;
1005 - epoxy;
1006 - diagonal joint;
1007 - multiple tongue and groove joint;
1008 - structural joint;
1101 - retired FRP plank;
1102 - tensile force;
1103 - polymer rope;
1104 - structure made of FRP elements
1105 - glue drop
1106 - FRP board
1107 - FRP plank
1201 - large piece of wind blade;
1301 - front view of the upper "comb" board 101;
1302 - side view of the upper "comb" board 101;
1303 - front view of the lower "comb" board 101;
1304 - front view of the lower "comb" board 101;
1305 - structure formed from "comb" boards 101;
1306 - elastic string;
1307 - retired FRP blade;
1308 - 3D printed element;
1309 - spacing "comb" board
1401 - string;
1402 - knot;
1403 - peg;
1404 - peg with hole;
1405 - retired FRP board;
1501 - concrete plate;
1502 - concrete plate;
1503 - vibration table;
1504 - FRP patches;
1505 - glue;
1506 - board 101 combined with cured concrete plate 1502;
1507 - temporary pressing for improved glue strength;
1508 - direction in which the beam should be placed on concrete plate 1501;
1509 - end of a wind turbine blade cut out;
1510 - element cut from a wind turbine blade;
1511 - double side reinforcement;
1512 - I-beam made of boards 101;
1513 - middle part of untypical I-beam;
1601 - coating of a bond-breaking substance;
1602 - dowel bar;
1603 - dowel bar;
1604 - dowel bar;
1605 - transmitting concrete:
1606 - rectangular peg;
1801 - chisel like tool;
1802 - cut;
1803 - drilling;
1804 - strong bar;
1805 - hole;
1806 - convex element;
1901 - measuring device;
1902 - connection;
1903 - control unit;
1904 - wireless connection;
1905 - wireless connection;
1906 - cutter;
1907 - carriage;
2001 - restricting (unflexible) string;
2002 - hinge;
2003 - flexible string;
2004 - axle;
2005 - triangular element of FRP;
2006 - claw screw;
2007 - triangular element of FRP;
2008 - folding structure;
2009 - folding structure;
2010 - snap-fit mechanism;
2011 - triangular element;
2012 - hinge;
2013 - hinge;
2014 - peg;
2015 - hole;
2016 - folding structure;
2017 - metal axle;
2018 - screw;
2019 - wedge;
2020 - folding structure;
2021 - snap-fit mechanism;
2022 - hinge;
2023 - internal hinge;
2024 - external hinge;
2025 - folding reinforcement structure;
2026 - square stick;
2027 - folding structure;
2101 - concrete arch;
2102 - rope;
2103 - polymer element;
2104-filter material;
2105 - compressing equipment.

### Preferred Embodiments of the Invention

The technical description of the present invention has been enhanced to include comprehensive specifications regarding the materials, precise dimensions, adhesives, types of screws, and the assembly and testing procedures for the upcycled FRP reinforcement. The FRP pieces, sourced from decommissioned structures such as wind turbine blades or other large FRP elements, are cut into flat sections approximately 20 mm thick, 2 meters long, and 0.5 meters wide. The bonding process employs high-strength epoxy adhesives, augmented with nanocomposite coatings for superior moisture resistance, and ultrasonic welding techniques to ensure robust joints. Screws/nails used in the assembly are typically 30-35 mm in length and 3 mm in diameter, coated with Zinc and epoxy to prevent corrosion and enhance durability. Detailed assembly procedures involve drilling precise holes, applying adhesives, and securing components with clamps until the adhesives cure. The production process is optimized for minimal energy consumption, using buzzsaw or advanced cutting methods like laser or waterjet cutting to reduce defects. Testing protocols include rigorous mechanical testing to assess tensile strength, bonding integrity, and resistance to delamination. Quality standards are maintained through strict adherence to industry benchmarks, ensuring that each reinforcement unit meets the highest standards of performance and reliability. This detailed technical framework not only ensures the robustness and effectiveness of the upcycled FRP reinforcement but also facilitates its adoption in various demanding construction environments.

According to the one embodiment of the invention a construction reinforcement, named by inventor "Stolat", suitable for use in concrete-based systems, comprising at least one board made of Fiber Reinforced Polymers (FRP), characterized in that the board is made of retired FRP and wherein the construction reinforcement comprises means for improving adhesion to concrete and the force transmission.

Preferably the means for improving adhesion to concrete and the force transmission are selected from the group comprising protruding elements 103, through holes 104, 110, grooves 315, 703, indentations, adhered loose materials and/or combination of them.

**Fig. 1****a** shows a construction reinforcement made of retired FRP boards 101. The procedure for preparing and installing the construction reinforcement can be carried out either on-site or in a workshop. Once the reinforcement is prepared, it should be transported to the construction site or mold where concrete will be poured on to this reinforcement. Alternatively, the reinforcement can be submerged in freshly mixed concrete. This method of reinforcement serves as an alternative to traditional steel rod rebar or pultruded Fiber Reinforced Polymer (FRP) rebar.

First, clean pieces of retired FRP boards 101 are cut, such as those cut from decommissioned windmill blades or other large FRP structures. These pieces should be approximately 20 mm thick, 2 meters long, and 1 meter wide. Next, through holes 104 with a diameter ranging from 10 to 100 mm are drilled (round or other shape). Drilling holes can weaken the strength of the reinforcement, so the holes should be spaced adequately apart, with a minimum distance of 100 mm from the edge or any other hole. To prevent water ingress over time, all cut edges of the FRP should be coated with a polymer, such as epoxy gelcoat preferably with hydrophobic additives.

Next, the prepared FRP boards 101 are glued together into a reinforcement 105 and the joints are reinforced by attaching fastening elements 102 with dimensions of 20 mm × 100 mm × 400 mm. Only two elements 102 are shown (Fig. 1a), but there can be many more depending on expected tensions. The narrow holes for screws 106 are drilled. Alternatively self-drilling screws or nails can be used by driving through the fastening elements 102 and into the FRP board 101 to enhance the adhesive bond and provide additional strength. Screws of 30-35 mm in length and 3 mm in diameter are suitable, and any type of popular screw head can be used. To prevent the corrosion and negative effect of humidity, the screws should be Zinc coated and covered with epoxy glue. Alternatively, gluing the fastening elements 102 without using screws is also effective, particularly if the glued surfaces are clamped until the adhesive cures. Alternatively, nanocomposite coatings can be used instead of epoxy coatings, which offer better protection against moisture and corrosion, increasing the durability of the reinforcement.

Additionally, FRP protruding elements 103 to the main surface of FRP board 101 using adhesive should be attached. Applying temporary pressure to these protruding elements 103 can help strengthen the adhesive bond. These protruding elements 103 are intended to enhance the bond between the construction reinforcement and the concrete.

If the reinforcement is manufactured off-site, it should be transported to the desired location. The flat bottom of the reinforcement has to be secured to a base layer, such as lean concrete, by gluing it or placing it on a fresh concrete base layer. To construct an entire structure or road with this construction reinforcement, multiple pieces should be assembled and inspected. Gelcoat should be applied to prevent moisture infiltration. It may be necessary to fix the reinforcement to the ground with pins.

Alternatively instead of flat bottom, elements 102 can be applied on the bottom side as well to strengthen the reinforcement, then securing the reinforcement 105 into fresh still-soft lean concrete base layer is recommended.

After a successful inspection, concrete or a similar construction material can be poured over the reinforcement. The final step involves pouring concrete, consisting of aggregates, water, and Portland cement (or alternatives to conventional concrete), in a 100 mm thick layer. The concrete should then be vibrated and cured. Additional layers of different types of modified concrete or asphalt may be applied later on top of the said 100 mm thick concrete layer.

**Fig. 1b** shows a similar reinforcement 105 made of two boards 101. Each board 101 is cut to obtain trapezoidal fastening elements 107 (20 mm thick, 200 mm long and 80 high, 5 deg inclination) and trapezoidal protruding pegs 108 and corresponding holes for the pegs 108 (20 mm thick, 80 mm long and 80 high, 5 deg inclination). Please note that the element 107 should be slightly off 90 degrees (like +3 and -3 deg) perpendicular line of board 101 connection. After cutting openings for elements 107, the edges of board 101 to be joined should be coated with glue and then boards 101 should be joined as shown by arrows 109 using 500 N force. It is necessary to coat the trapezoidal element 107 and the holes for the element 107 with glue and hammer into the opening. Then, it should be ensured that the element 107 protrudes from the lower part of board 101. Additional narrow trapezoidal protruding pegs 108 are to make stronger connection of the reinforcement 105 to concrete. The pegs 108 and their holes should also be coated with glue and the pegs 108 should be hammered into the holes. All the elements 107 and the pegs 108 are made of retired FRP. They are glued to the board 101 and hammered into 101. The element 107 has double function as a connecting element and as a protruding element for better connection with concrete and passing forces to and from reinforcement, wherein the element 108 has a single function - just a strong protruding element which will prevent delamination of the board 101 as protruding element 103 may do if cutting forces are too strong.

After anti moisture coating and glue cures, the reinforcement 105 from fig. 1b is ready to be secured to the ground and poured with concrete. Such reinforcement 105 can be also used as stay-in-place formwork.

**Figure 2a** shows the alternative way to connect the FRP reinforcements which involves preparing two flat pieces of retired FRP board and milling the joining planes as shown marked with three lines on the lower FRP board 101, mirroring it with the upper FRP board 101 (Fig. 2a). The size of the pieces should be 20 mm thick, 2 m long, and 1 m wide. Next, the epoxy glue should be added to the surfaces to be joined, and a glued joint 202 should be pressed with a force of 1 kN, as shown by the arrows, according to the standard procedure for woodworking as it is shown in **Figure 2b****.** The combination of two FRP 101 boards results in a joined reinforcement 201.

**Preferably** the protruding elements 103 are selected from the group comprising screws 106, 902, 903, pegs 108, 1004, 1403, 1404, 1607, bolts 1001, 1002, 1003, dowels, plugs 2014, expansion anchors, fasteners made of retired FRP 102, 504, strings 301, 313, 1103, 1401, strands, knots 1402, retired fishing nets 302, bottle cups 303, polymer tines 307, rebars 322, FRP chunks 702, convex elements 1008, 1806, and/or combination of them.

**As shown in** **Fig. 3a****,** long pieces of polymer string (one or many strands) are glued to the board 101 to improve the connection between the concrete and the reinforcement. These strings can be attached at various angles relative to each other, including at 90 degrees. The procedure involves preparing an FRP board 101 of appropriate size, which can be made by joining together several smaller boards. A proposed size is 20 mm thick, 2 m long, and 1 m wide. Long pieces of polymer string 301, which can be rope (not biological origin to avoid swell) preferably of polymer material, are attached to the side of the board 101, which will later touch the concrete. If both sides of the board 101 will be touching concrete, the strings should be glued to both sides.

Although not shown in Fig. 3a, the reinforcement should be placed on a still-soft lean concrete base or it can be secured by gluing to cured flat base.

**Alternatively,** instead of string, it is possible to use the retired fishing net 302 for strengthening bond between concrete and reinforcement (see **fig. 3b**). Fishing nets are known for water and alkali resistance so retired fishing nets are good choice from ecological, economical perspective and reinforced concrete longevity.

**Alternatively,** other elements can strengthen the bond between concrete and the construction reinforcement. For example in **fig 3c**, after preparing an retired FRP board 101 of decent size, which can be made by joining together several smaller boards, one can glue (using epoxy or thermoplastic glue) retired plastic bottle caps 303 (or other end of life small polymer elements) to the board 101 and preferably secure them with the one screw 106 (or nail) to the board 101 to provide strong pressing force for glue curing. These caps enhance the connection between concrete and the board 101. Although only two such caps are visible in Fig. 3c, many more can be attached for stronger bonding between concrete and the board 101. Alternative to plastic bottle caps one can use mass produced small polymer elements nailed or screwed to 101 with or without glue.

Preferably the through holes 104 having dimensions in the range from 10 to 900 mm, wherein the drilling angle is in the range from 40 to 140 degrees can be used. Additionally round, oval or other shape through holes 110 with shallow 2 mm indentations 701 at its edge (easy to cut with saw) can be used. All freshly cut FRP should be protected with gelcoat or epoxy glue. A flat pieces of PET bottle 304 should be prepared with a shape similar to a rectangle, measuring 50 mm by 30 mm in this example. It is necessary to cut the sides of 304 into many polymer tines 307, such as 15 teeth on each longer side resulting in element 305. Then the tines should be bent upward on both sides, as shown in Fig. 3c, 306. It is necessary to glue the "toothed rectangle" 306 to the board 101 using epoxy glue or other glue dedicated to PET, but leaving the "teeth" free, attaching only the middle part of the rectangle 306 to the board 101. Although only two glued toothed rectangles 306 are shown in Fig. 3c, many more can be attached to strengthen bonding between concrete and the board 101. Innovative shapes, such as three-dimensional composite meshes, can also be used to reinforce concrete, offering better mechanical properties and greater design flexibility.

The construction reinforcement should be inspected and preferably gel coated to prevent moisture penetration. After a positive inspection, concrete or similar construction material can be poured on such reinforcement.

Preferably the adhered loose materials ale selected from the group comprising sand 308, polymer elements, FRP elements, ground FRP dust, epoxy resin 310, gravel, aggregates, quartz, broken glass, perlite, ceramic, corundum, polyurethane powder, pumice, silicon carbide, and/or combination of them.

**Another example** of enhancing connection with concrete is presented in **fig. 3d****.** The side of the board 101, which is in contact with concrete should be covered with a thin layer of epoxy glue. It is recommended to sprinkle the adhesive with coarse sand 308 (size 0.5 to 1 mm) and wait for the adhesive to harden. This step can also be applied to the bottom side of this reinforcement to improve the bond between this construction reinforcement and the base in example lean concrete. The unattached sand should be blown away with air or the reinforcement should be turned upside down so that the loose sand falls off. Coarse materials other than sand for example gravel, perlite, polymer elements, especially sand-sized pieces of retired FRP, broken ceramics or glass, and/or combination of them can be used as well.

**Different** way of improving connection is presented in **fig. 3e****,** where the board 101 painted with epoxy is made rough with a brush 311 by vertical hitting or a roller 312 by rolling. The rough area is marked as 310, while the glossy epoxy area not yet made rough with brush hitting or roller is marked as 309. Hitting vertically with brush or rolling with roller makes the epoxy surface rough for better grip with concrete.

**Figure 3f** shows a retired FRP board 101 with improved grip for concrete with thermoplastic and similar technologies. Due to easy robotisation it is very cheap and can be done with not only flat boards.

A reinforcement board 101 measuring 2 meter by 1 meter by 20 millimeters is prepared. The surfaces of the board must be clean and free from any traces of oils or contaminants to ensure good adhesion. Using a robotized control unit, the specific areas where such connection enhancement is desired are identified and memorized by robot control unit. A large 3D printer or similar robotic system is employed to apply the temporary fluid material. The extrusion head 314 of the printer produces a string of polymer 313 using technologies such as Fused Deposition Modeling (FDM), Fused Filament Fabrication (FFF), UV or light-activated resin, laser sintering, or evaporative adhesion. The extrusion head can be operated manually or automatically by the robotic system and must be capable of moving relative to the FRP board 101 to apply the thermoplastic material in the designated areas. Optionally, the fresh thermoplastic material can be coated with sand or a similar substance, as is shown in Figure 3d.

**Different way** of improving bonding of reinforcement with concrete is shown in **fig. 3g** It is a family of plunging methods. There can be seen a milling head 316 making grooves 315 of desired length of 5 mm wide and 3 mm deep in the board 101. Similar rows can be obtained using press 321, plasma, laser, waterjet, a rotating saw 320 or a grooving hook 319. Raised edges 318 of the row can be a result of pressing FRP material or additional epoxy glue added after the grooving 317. Using wire wheel brush 331, rasp 332 and sandpaper 333 depicted on the right and sanding process (not on illustration) are good methods to increase the roughness of surface of FRP board for better adhesion to concrete.

**Figures 3h****-i** show the hybrid of the board 101 glued with steel or FRP pultruded rebar 322. Fig. 3h on the left shows three rebars 322 glued to the board 101, wherein on the right shows two pultruded FRP rebars 322 joined together by two glued rectangular boards 101 each with semicircular groove 334 (matching size of diameter of 322) making much longer hybrid reinforcement. One must put the ends of rebars 322 in the grove 334, add glue and close with the other 101 and temporary press together. Fig. 3i on the left shows the board 101 with a large oval through hole 110 with several 3 mm indentations 701 on the edge of the oval to improve bonding with the concrete. The oval through hole 110 has two holes 325 for rebar 322, rebar 322 is glued and pressed into these holes. Fig. 3i on the right shows solution to pultruded FRP rebar 322 which cannot be bended at the ends, one end is finished with two glued triangular boards 101 with semicircular groove 334 each, the other is finished with two glued rectangular boards 101 also with semicircular groves 334 closer to one end of 101, so the other end is pultruding a lot at the right angle from the rebar 322. Such ends help in force transmission.

**Fig. 3j** shows a foldable, snap-fit reinforcement made of the lower and the upper board 101 with rectangular holes 323 matching snap-fits on the ends of the H-board 324. The stabilizing triangles 326 are made of retired FRP and are glued to the H-board 324, thanks to the triangles 326 after inserting snap-fits to holes 323 the whole spatial reinforcement is stable. Ways for improving bonding to concrete of this reinforcement is not shown, but several ways disclosed in this document might be used.

**Fig. 3k** shows another example of improved bonding to concrete using thin biscuit joints 327 made from FRP or other strong material. On a retired FRP board 101 1000 mm long, 100 mm wide and 20 mm thick one should cut multiple 4 mm incisions 328 of 2 mm wide as shown in fig. 3k. Into these incisions 328 biscuit joints 327 having dimensions of 30 × 40 × 2 mm should be glued. The spacing between them should be from 10 to 300 mm. Such reinforcement will be specially good for the tensile strength of the board 101.

**Fig. 3l** shows stirrup or tie made of four boards 101 with dimensions 300 × 40 × 10 mm. They are glued together and nailed with nailer gun (nail not visible). Four rebars (steel or pultruded FRP) 322 are attached by zip ties 330 to the said stirrup/tie. Such stirrup/tie will bond well with concrete and also transfer forces because of its shape - short boards 101 are joined at right angles.

**Fig. 3m** on the left shows similar stirrup/tie where rebars 322 are fixed via flexible clamps 329, which are glued to stirrup/tie. Also two upper rebars 322 are pressed in trapezoidal openings in board 101. On the right is circular stirrup (spiral) made of circular board 101 cut from round retired FRP pressure gas container, four rebar 322 are attached via flexible clamps 329.

**Fig. 3n** shows upper board 101 which shape resembles letter H, made of 1000 × 10 × 40 mm board 101 and width is machined symmetrically 5 mm off from both sides to be 30 mm wide. This shape enhances transfer of forces between reinforcement and concrete. Lower 101 board with short perpendicular 101 bords at its ends is similar to upper board but made of three glued together boards 101 instead of one.

Preferably the boards 101 are butt jointed or at least partially overlapping. The butt joint is a straight joint, a diagonal joint, a structural diagonal joint 1006, a multiple tongue and groove joint 1007 or a structural joint 1008.

**If at least one board** is not substantially flat, but angled at one edge, the procedure involves preparing retired FRP boards, ensuring that at least one is not completely flat (**Fig. 4**). The size should be 20mm thick, 1m long, and 0.5m wide. Cut the edge of the board 101 for a contact area 401. The angled FRP board 101 and the flat FRP board 101 should be glued together at the contact area 401 as shown in Fig. 4 and additionally screws (30mm long, 3 mm diameter, one per every 100mm of joint) should be used to strengthen the glue bond. Alternatively nails or just temporary clamping force can be used. Any screw/nail should be covered with epoxy glue to prevent moisture and corrosion. One should prevent pockets of air under said reinforcement when pouring concrete for example with small holes for air escape. Although preparing the surface for better bonding of this construction reinforcement and concrete is not shown, it can be done in any ways disclosed in this document.

Preferably the boards 101 are jointed by adhesive and/or by other means, selected from the group comprising dovetail, pegs 108, 1004, 1403, 1404, dowels, plugs 2014, expansion anchors, bolts 1001, 1002, 1003, screws 106, 902, 903, and/or combination of them.

**The procedure** of preparing large construction reinforcement from many smaller flat pieces, as shown in **Fig. 5** involves preparing boards 101 and glueing them together face to face with epoxy or another polymer adhesive, applying a force of 100-500 N for good adhesion. Pieces like fastening elements 102 and fasteners of different shapes 504 should be attached using glue and additionally screws or nails (106, 903) to attach any two boards 101. Any screw should be covered with epoxy glue to prevent moisture and corrosion. Through holes 104 of diameter 20-100 mm are drilled in the board 101 to strengthen the connection of this construction reinforcement with the concrete that will be poured on it. The freshly cut sides of the FRP should be coated with hydrophobic epoxy or another polymer glue to prevent moisture penetration.

Fastening FRP elements 102 are attached with glue and screws to the side that will later be joined to another module such as 502 (a module of multiple joint boards 101) or to 503 (another module of multiple joint boards 101). The modules should be inspected and any metal or unprotected FRP should be covered with an anti-moisture coating like epoxy with 1% graphene. Elements 501 are prepared to pull the large module 502 with a crane and ropes 505. An element 506 is an alternative mean for this purpose, it is easier to handle rope on 506 than using 501.

**Preferably the construction** reinforcement can be arranged in the two-deck structure (see **fig. 6a****-c**). To obtain the double-deck construction reinforcement, first the lower board 101 should be prepared, as shown in Fig. 2. The dimensions should be 20 mm × 2 m × 1 m. **Fig. 6a** shows the trapezoidal cross-section of FRP brackets 601 with height of 200 mm, length of 2 m and thickness of 20 mm, angled at around 45 degrees which should be glued to the lower board 101, using temporary force to strengthen the glue binding or strengthening with screws or nails. Epoxy glue is suitable for this. A row of such brackets 601 should be placed every 200 mm. It is important that all the brackets 601 stand out at exactly the same height.

All the upper areas of the trapezoidal brackets 601 connected with the lower board 101 should be covered with epoxy glue when the upper board 101 is placed on them and pressed. Screws or nails may also be used but are not shown. After glue and anti-moisture coating cures than fresh concrete 602 is added. Please note that holes and other means of improving bonding with concrete are not shown for clarity.

Preferably the boards 101 are arranged in at least two parallel planes connected by FRP brackets 601, wherein the axial distance of the planes is in the range from 20 mm to 900 mm.

**The double-deck** (or multi-deck) construction reinforcement will also work well for non-road applications, such as vertical construction components. For example as shown in **fig. 6b**, it can be used as construction reinforcement for a rectangular pillar sized 300 mm × (300-1000 mm) and 4 m long.

**Figure 6b** shows an example of a spatial (non-flat) reinforcement made from flat retired FRP boards 101. Although glue is not shown in the figure, it should be applied wherever the boards are joined, and metal screws/nails 106 should be protected against moisture/corrosion with zinc layer and hydrophobic coating. Alternatively nonmetallic screws/nails should be used.

The procedure involves preparing two side boards 101 (20 mm thick, 1 m wide and 2 m long) secured with glue and screws to the lower board 101 (20 mm thick, 2 m long, and 1 m wide). Glue should be applied, 2 mm holes drilled, and screws 106 driven in (alternative are nails installed with nailer). Then, the partial assembly should be turned upside down so that the lower board 101 is on the bottom, after cutting the edges of a diagonal FRP plate 101 (around 45 degrees, to fit), place it diagonally, use glue and screws/nails 106 to fix it. The upper board 101 should be glued on top, and then fastened with screws or nails 106. The assembly should be inspected for any risk of moisture entrance, and any exposed areas should be covered with coating. After allowing the adhesive and coatingto cure, the unit will be ready to serve as a girder type of reinforcement or to be fully submerged in the concrete 602 as in fig. 6b. Any previously shown methods for strengthening the bond with concrete 602 can be used, although they are not shown in the figure for clarity.

**The procedure** for making a road (or a slab or a ceiling) with a double deck of construction reinforcements has been depicted in fig. 6c. First the lower aggregate and lean concrete should be prepared as a base. A flat lower FRP board 101 having dimensions of 20 mm × 5 m × 2 m with through holes of 30-50 mm should be prepared, similarly preparing the upper board 101. The 100 mm wide boards 101 should be glued and attached to the lower board 101 with screws 106. Screws 608 should be used for stronger bonding with concrete (one per every 100 mm square). Then cover all exposed FRP and screw heads with a moisture barrier coating. Cover all top areas of the board 601 with epoxy adhesive to bond to the upper board 101 (see Figure 6c). The upper board 101 should be placed on the freshly glued areas of the board 101 and heavy masses should be applied to induce a temporary force of 300-900 N per square meter for proper glue bonding or use screws or nails. Temporary force-inducing objects should then be removed. If there is no temporary force, then claw screws 903 should be screwed into the upper layer of the upper board 101 (5 times less than the screws 604). An anti-moisture coating should be added. The adhesive should be cured and reinforcement should be fixed to base. Concrete 602 consisting of aggregates, water, and Portland cement (or alternatives) should be poured in a 100mm thick layer inside the double layer and another 100mm thick layer on top of the construction reinforcement. The next steps are vibrating and curing the concrete. For the top layer 603, modified asphalt 20 mm thick should be used on top of the poured concrete if it is road build.

**Figure 7a** shows an example of an FRP rectangular board 101 prepared for better grip with concrete. The procedure involves preparing a clean retired FRP rectangular board 101 that is 20 mm thick, 20-50 mm wide, and several meters long (shown short version in Fig. 7a), triangle, rhombus or trapezoid cross section is also good alternative to rectangle. Then, cutting operations are performed on the edge of the board using a knife (hand-driven or machine-driven), buzzsaw as depicted, threading head, lathe or similar tool or kind of saw, water jet cutter, plasma cutter etc. Preferably, each indentation 701 is made of 2 cuts at an angle of 15-120 degrees between them, and 3 mm deep. Alternatively, a special mechanized V-shaped knife or chisel can be used to perform this operation in a single cut. Turning the board 101 in lathe may help to mechanize this process.

Next, grooves 703, around 5 mm deep and with a diameter from 5 to 12 mm, are made in the side of the board 101. After drilling, a thin layer of epoxy with hydrophobic additives should be applied to protect against moisture. Small chunks 702 of FRP, for example the residues from the cutting of indentations 701, should be glued to the side of the board 101 with epoxy containing hydrophobic additives. All FRP chunks should be covered with this epoxy. For even better bonding use sand, as is shown in fig. 3c, on fresh epoxy.

After the protective polymer (or glue) has cured, the element will be much better prepared to become concrete reinforcement, as the forces from concrete to FRP and vice versa will be transferred effectively. It is recommended that such the board 101 be used as straight replacement of traditional rebar from steel or pultruded FRP. Please note that on fig. 7a are shown only two of four edges with indentations 701 for clarity, recommended are indentations on all four edges.

**Fig. 7b** **shows** at top a process of a mass production of an edges cut board 101. First a large retired FRP board 101 (20 mm × 3 m × 10 m) is cut by a battery of parallel rotating saws 706 into several boards 704 with cross-section dimensions of 20 × 30 mm. Saw dust from cutting is collected and transported with air by the duct system 705. Boards 704 are immediately processed by a battery of rotating thread cutters 707 to make indentations 701 on the boards 704 making the edges cut boards 101. Dust from this operation is also collected and transported with air by the duct system 705. Boards 101 are sprinkled by a battery of sprinklers 708 with low viscosity glue. Immediately afterwards wet with the glue, the boards 101 are covered with a dust from 705 with a battery of saw dust heads 709. Some of saw dust is attached to the boards 101 and the not attached dust is redirected back to 709. Alternative process of production of 101 board with indentations as on fig. 7a is at the bottom of fig. 7b. Trapezoidal screw is turning the board 101 around and forward to rotating saw 706 making indentations 701 on four edges of 101.

**In** **fig. 8** another way of improving bonding is shown. Two wavy edges of a board 101 improves the grip with concrete. It has dimensions of 20 mm thick, 1 m long and 20-40 mm wide. To make the wavy board 101, the straight board 101 should be prepared to be cut in wavy shapes. Cut wavy edges 802 (oscillating 3-7 mm from strait path) as in fig. 8. The numbering 803 shows the planned wavy path to be cut. A narrow band saw 801 can be replaced with other thin cutting tool that allows wave cutting. It can also be a saw cutter, an oscillating saw, a cutout saw, a jigsaw, laser, plasma, a waterjet and similar cutting tool.

Wavy edges improve grip of concrete transferring forces. Finally, the board 101 can be painted with anti-moisture paint. To further improve the adhesion of the joint to the concrete, it is recommended to use other methods disclosed in this application. When the paint cures the board 101 is ready to be used as a reinforcement for concrete.

**Fig.9** **shows** how bear claw screws can be used for improving connection between concrete and FRP reinforcement, it also counteracts delamination. Black thick dash and black drops represent the epoxy glue 1005 or other polymer glue.

To prepare the upper board of retired FRP 101 (10 mm × 2m × 1 m) for connection with the lower board 101 and subsequent contact with concrete or similar material, first drill a narrow hole 901, approximately 3 mm in diameter, for the bear claw screw 902. Fill the drilled hole with epoxy 1005 containing anti-moisture additives, ensuring sufficient epoxy to allow overflow upon driving in the bear claw screw 902, as indicated by small arrows. Then drive the screw 902 into the hole 901, ensuring that the outside diameter of thread is 4 mm. Use any known type of screw head, with Hex and Torx being preferred for their speed and reliability. The epoxy 1005 in the hole 901 serves to protect the FRP board 101 from moisture and additionally improve the strength. Fully cover the installed bear claw screw 902 with epoxy 1005 containing anti-moisture additives. Alternatively, consider using a new bear claw screw 903, where only a portion (approximately 40%) of its length, starting from the sharp point, is threaded. This aids in applying clamping force between the boards 101, enhancing their bond, still giving strong grip with concrete and counteracting delamination. Alternative is bear claw nail preferably driven in by nailer (nail gun).

For the bottom board of retired FRP 101 note that the bottom side depicted in Fig. 9 is not intended for improved contact with concrete (no protruding screw heads). However, if other bear claw screws were protruding out of the board 101 downwards, it would enhance its connection with concrete at the bottom.

**Fig 10a** shows the procedure for joining two retired FRP boards 101 "side to side" for larger size reinforcement which involves either making holes first, and applying epoxy 1005 to the "side to side" areas later, or alternatively applying epoxy 1005 to the areas, then joining and compressing, and finally making holes for the coming screws and/or bolts and/or nails 1001, 1002, 1003 and pegs 1004 The holes should be 3 mm in diameter, as shown in Fig. 9. The screw 1001 should be fixed from both sides, especially when longevity is needed and corrosion is a concern consider non-metal or non-corroding screws. Epoxy 1005 with anti-moisture ingredients should be added to protect the metal screw 1001. For better connection with concrete, the protruding tabs of each head of fixing screw 1001 should be utilized. One or more drops of epoxy 1005 should be put into the hole before screwing the screw 1002. Various screw heads are possible; the example is shown in Fig. 9 wherein the protruding hexagonal type will strengthen the grip with concrete after it is added. Then, the screw 1003 should be fixed from one side, as shown from the side of the board 101, and the nut should be fixed on the other (upper) side of the board 101. Strong compressive force should be applied for better glue grip, but excessive force should be avoided to prevent damage to 101. The bear claw screw 903 should be fixed as described in Fig. 9. A drop of epoxy 1005 should be put into the hole before fixing polymer peg 1004. Consider non-metallic screw/bolts when corrosion or electromagnetic field is an issue. Symmetrical joint solution shown in Fig. 10b will not warp when tensile stress is applied.

**Figure 10b** shows an example of a non-warping joint of two retired FRP boards 101 "face to face" glued for larger size reinforcement for concrete. Several joint types are shown, similar to those in Fig. 10a, and their function is to strengthen the boards against delamination when strong shearing forces are applied. Two additional boards 101 are used compared to embodiment in **Fig. 10a****.** Here, only plastic pegs 1004 (pegs with a 6 mm diameter) and screws with nuts 1003 (6 mm) are proposed.

The procedure involves preparing the first board 101 (10 mm thick and 500 mm long and wide as 1002) and the second board101 (20 mm thick, 2 m wide and several meters long) by cleaning the surfaces to be glued. It is suggested to use epoxy with a 1% graphene additive for moisture protection. Then, place one (bottom) 101, apply epoxy 1005 to it, and position both the second boards 101 face to face on the fresh epoxy 1005 on the bottom board 101. Ensure that the epoxy 1005 is applied between the boards 101 as well. Glue the upper board 101 to this assembly and drill 6 mm holes. Although only 4 holes for dowels and pegs are shown, for example for a 2-meter-long joint 20 holes are recommended. When epoxy 1005 has not yet cured, insert polymer pegs 1004 and bolts 1003, and apply epoxy 1005 for moisture protection. Secure nuts to the bolts 1003 for strong clamping, similar to the process used with wood. Alternatively, holes can be drilled first and the gluing performed afterward. Instead of bolts 1003 and nuts, any of the joints depicted in Fig. 10 can be used, as well as non-threaded or threaded polymer pegs 1004 with external clamping force during adhesive curing.

**Figures 10c****-e** show examples of other non-warping joints, namely a diagonal joint 1006, a multiple tongue and groove joint 1007, and a structural joint 1008, of two retired FRP boards 101. One must first cut the edges of left and right boards 101 to be joined, as in each figure 10c-e, where the cut edges are mirrored on the corresponding edges. Then apply epoxy 1005 to the surfaces to be joint, a temporary clamping force 109 of 500 N should be induced to allow the epoxy 1005 to flow out. Remove clamping force 109 once the epoxy 1005 has cured.

After inspecting this joint, the unit is ready to become a large flat reinforcement for concrete.

After all epoxy 1005 has cured, this larger reinforcement, as shown in Figs. 10a-e, is ready for concrete to be poured onto it, or the reinforcement can be placed into fresh, soft concrete for the desired reinforcement function. Other disclosed in this application ways of strengthening grip with concrete are not shown in fig.10 but should be considered.

**Figure 11a** shows an example of retired FRP reinforcement specifically designed for in factory concrete module production. The reinforcement unit consists of 7 retired FRP boards 101 to be prestressed before pouring concrete, similar to the method used with steel rebar concrete units. The reinforcement is pulled from both ends by a tensile force 1102 (indicated by black arrows) of 7 kN. This force should not break the reinforcement, but after the concrete cures and the tensile force is released, it will impart significant compressive force to the concrete.

The procedure for making prestressed modules with the described reinforcement involves making holes 104 in boards 101 and covering the freshly cut resin with polymer to prevent moisture. Seven boards 101 are then placed as shown in figure 11a, glued, and screwed to four retired FRP planks 1101 with screws or nails, ensuring the screws are covered for moisture protection. Once the epoxy cures, the unit is turned upside down, and three additional retired FRP planks 1101 are placed as shown in figure 11a, glued, and screwed to the board 101, again covering the screws/nails for moisture protection. After waiting for the epoxy to cure, the prepared unit is placed on a stable vibration table (or without a vibration table) in the concrete units factory. Ropes are used to pull seven boards 101 with a total tensile strength of 7 kN, applying 1 kN to each board. The unit is inspected for any cracks, protected from moisture with coating. The desired amount of concrete is poured onto the unit, using the vibration table to enhance concrete quality, and the concrete is smoothed with appropriate tools. After allowing the concrete to cure, the force is deactivated, the pulling ropes are removed, and the concrete-reinforced unit is removed for designed use.

**Figure 11b** shows two rectangular boards 101 fixed with glue and screws/nails with two retired FRP planks 1101 (similar to Fig. 11a). Again 1 kN of tensile strength should be applied at ends of each 101. After protecting this reinforcement unit with anti-moisture paint, and after it cures concrete should be poured, vibrated on this reinforcement unit similar to situation described at fig.11a. One may consider replacing the flat board 101 from fig. 1a with this shown at fig. 11b in some instances.

**Figure 11c** discloses a variation of module from fig. 11b which is not prestressed but foldable. Fig. 11c shows alternative to beam reinforcement, which is foldable. Two modules 1104 from fig. 11b are one over the other. Polymer rope 1103, preferably retired marine rope or made of UHMWPE, or PP or PET tape is tightly wrapped around said two modules and glued with drops of epoxy 1005 (alternative to epoxy - ultrasonic welding might be used). Between the two modules 1104, there are two boards made of retired FRP - 1106 with through holes for better bonding with concrete and a board 1107 also of retired FRP. The role of the boards 1106 and 1107 is to space two said modules 1104 and springiness of FRP elements counteracting with the rope allows to easy dismount the spatial arrangement shown in fig. 11c into flat elements because the boards 1106 and 1107 are not permanently connected with the rest of elements, only the springiness of the arrangement keeps it in place for the coming concrete. The first board 1106 is 250 mm wide, the second board 1107 is 30 mm wide and both are 10 mm thick and 300 mm high. Important to note is that the rope 1103 will work as stirrups in traditional rebar reinforcement. Ease of transportation of flat reinforcement is a strong advantage, also ease of folding up back into spatial arrangement shown in fig. 11c. One may use double 1107 for stability if needed. This beam reinforcement may work better in some cases when turned 90 degrees, on its side.

**Figure 12** shows top view of half of circular reinforcement made from many large pieces of retired wind blades 1201. If height of 2 meters of reinforcement is required, than cut this length of blades and glue them together with multiple L-shaped boards 101 cut from other wind blades. When full 360 degrees reinforcement is done (consider other disclosed ways of enhancing bonding with concrete) it will be strong enough to reinforce wind generator foundation or some other demanding concrete construction.

Preferably the board 101 is substantially flat or has a shape selected from comb, angled board, U-shaped board, L-shaped board, T-shaped board.

**The construction** reinforcement can be also prepared from "comb" boards. For example from six "comb" boards 101 made of retired FRP (see **Fig. 13a**). The dimensions should be 20 mm in thickness, 600 mm in length, and 60 mm in width. Each "comb" side opening should be 30 mm long and 20 mm wide. Holes 104 with a diameter of 5-15 mm as shown in Fig. 13a should be prepared. 1301 is a front view and 1302 is a side view of the upper "comb" board 101. 1303 is a front view and 1304 is a side view of the lower "comb" board 101.

All FRP cuts should be for longevity covered with an anti-moisture coating, such as epoxy with hydrophobic additives like 1% graphene. The lower "comb" board 101 should be placed in parallel with the openings facing upward and the areas to be in contact with the upper "comb" board 101 should be covered with glue. Similarly, the same areas on the upper "comb" board should be covered with glue. Epoxy glue is suitable for this purpose. The upper "combs" should be inserted into the slots of the lower "combs" to form the structure 1305 of "comb" boards 101.

**Figs. 13 b-c** show folding reinforcement where three FRP rectangular boards 101 are connected by a string 1307 (preferably elastic like retired rubber) glued to each board 101. Function of such the string 1307 is to make setting up the reinforcement structure fast and convenient. Folding structure is easier for transportation and can be set up from shown in fig 13b to shown in fig. 13c easily on site with only hands and hammer. Just two "comb" retired FRP boards 1309 with glued 2 blades 1307 also made from retired FRP are put down on stretched unit of three boards 101 and hammered down. Function of the "comb" boards 1309 and the elastic string 1306 is to space the boards 101 as designed from each other and keep the unit together when concrete is poured and make it convenient for workers on site. Blades 1307 glued to 1309 are to hammer the whole reinforcement into the ground. Ideally glue should not be needed at construction site for this reinforcement as poured concrete will set this unit still as shown in fig. 13c but glue might be used for strengthening this reinforcement before concrete is poured. Consider using anti-moisture paint in this reinforcement. If the ground is too hard to hammer blades in, than shorter, blunt blades should be glued to the ground or left for gravity to keep it in place.

**Similar** to fig. 13b-c is the example shown in **fig.13d****.** There are three FRP rectangular boards 101, but these are joined by pressing into trapezoidal openings in two 3D printed elements 1308 (these can also be made of retired FRP or as a hybrid of 3D printing on retired FRP or as moulded plastic element). The function of the elements 1308 is to space the boards 101 at the designed distance from each other and improve the force transfer, trapezoidal openings in 1308 help to secure 101 tightly in them. Fig. 13d shows a reinforcement that is easy to transport and easy to assemble, without tools and without additional fasteners at the construction site.

**Figure 14a** shows a concrete reinforcement made from a retired FRP board 101 with improved grip with holes 104 and a string 1401 threaded through those holes.

The procedure for manufacturing concrete reinforcement from retired FRP boards 101, with improved connection using holes 104 and threaded string 1401, begins by preparing a reinforcement board 101. It is essential to ensure the surfaces are clean and free of any oils to promote good adhesion. Through holes 104 (10 mm diameter) are then drilled in the board as required. Anti-moisture paint (functioning also as a glue for string) is applied to the surfaces exposed by cutting or drilling. A string 1401, similar to the long pieces of the polymer string 301 from Fig. 3a, is threaded through the holes 104. Knots 1402 are used at the ends of the string 1401 to ensure it is tightly threaded, and glue is applied to further strengthen the grip between the concrete and the reinforcement. The reinforcement is now ready for concrete to be poured onto it or for placement and vibration into fresh concrete.

**Figure 14b** shows a concrete reinforcement made from a retired FRP board 101 with improved grip with holes 104, pegs 1403, pegs with hole 1404 and a string 1401 threaded through holes 104 and additional pegs 1403, 1404, preferably from FRP for stronger grip on string 1401. Pegs 1403 are used to provide the string 1401 glued to end of 1403 does not fall off. Alternatively, pegs 1404 with hole can be used for stronger connection to the string 1401. Fig. 14a shows a flat string on the board 101, while fig. 14b adds a vertical dimension to fig.14a.

**Figure 14c** shows another example of similar concrete reinforcement made from retired FRP board 101 with improved string grip with vertical dimension threaded through the holes and around the board 101. The procedure starts with the preparation of the reinforcement board 101 which can be procured using the shape of a wind blade with a small amount of cutting. Surfaces should be cleaned thoroughly, with any traces of oils removed for good adhesion. Holes 104 of 10 mm diameter are drilled in the board 101 as needed, and semicircular grooves of 3 mm diameter have been prepared on the edges of the board 101 so that the string 1401 does not move. Anti-moisture paint is applied to the surfaces exposed by cutting or drilling. A 4 mm thick, water and alkali-resistant polymer string is threaded through the holes 104 and around the board 101 in those semicircular or rectangular grooves, as shown in fig. 14c. Knots 1402 are used at the ends of the string to ensure it is tightly threaded, and glue is applied especially to the contact points of the strings 1401 and the board 101. Once the glue cures, the reinforcement is ready for concrete to be poured onto it or for placement and vibration into fresh concrete. The retired FRP board 1405 is depicted to show that similar spatial reinforcement is possible, but without using the string.

**Figures 15a****-h** show a cross-sectional view of a bridge (or another supported horizontal construction element) beam/girder reinforcement constructed from retired FRP boards 101. Such reinforcement can also be used fully submerged in concrete like depicted in fig. 15g. Element in Fig. 15a shows an inverted beam before placement on wet concrete, positioned on a vibration table 1503 to enhance concrete quality. Element in Fig. 15b illustrates a bridge beam with a concrete deck on the top. Elements in Fig. 15c and Fig. 15d similarly represent other types of beams, demonstrating the versatility in creating various beam shapes from retired FRP boards 101. Fig. 15e shows making of an I-beam made from retired FRP boards 101, where fig. 15f-g shows examples of use of such I-beam with concrete. Fig. 15h shows side view of untypical I-beam with slightly curved bottom part; fig. 15i shows beam/grinder similar to fig. 15d but simpler by different attachment to concrete.

Another aspect of the invention is a construction element comprising the construction reinforcement embedded in concrete of the thickness in the range from 20 mm to 9900 mm, wherein the concrete comprises aggregates, water and cement, and wherein the cement is selected from the group comprising Portland cement, geopolymers, fly ashes, blast furnace slag, belite cement, cement from agricultural ashes, aluminous cement, pozzolanic cement, silica fume, metakaolin, polymers functioning as binder and and/or any combination of them.

Another aspect of the invention is a method for obtaining the construction element defined above, which comprises the following steps: a) placing in the board 101 the means for improving adhesion to concrete and the force transmission are selected from the group comprising: screws 106, 902, 903, pegs 108, 1004, 1403, 1404, bolts 1001, 1002, 1003, dowels, plugs 2014, expansion anchors, fasteners made of retired FRP 102, 504, strings 301, 313, 1103, 1401, strands, knots 1402, retired fishing nets 302, bottle cups 303, polymer tines 307, rebars 322, FRP chunks 702, convex elements 1008, 1607, 1806, grooves 315, 703, indentations 701, adhered loose materials selected from the group comprising sand 308, polymer elements, FRP elements, ground FRP dust, epoxy resin 310, gravel, aggregates, quartz, broken glass, perlite, ceramic, corundum, polyurethane powder, pumice, silicon carbide, and/or combination of them and/or drilling the through holes 104, 110 in the boards 101, in the distance not less than 10 mm from the edges of the board 101 and from any other hole 104, 110; b) optionally, covering all uncoated cut edges of the board 101 with polymer; c) jointing of boards 101; d) pouring the reinforcement construction obtained in steps a)-c) with concrete material with a thickness of at least 40 mm or dipping the reinforcement construction into fresh concrete material with a thickness of at least 40 mm; e) optionally vibrating and curing the concrete at a time of at least 2 hours (with fast curing concrete), preferably much more.

**Figure 15a** shows soft, uncured concrete for concrete plate 1501, waiting on vibration table 1503 for concrete reinforcement. Fig. 15b shows a cured top concrete plate 1502. Additional elements depicted in Figs.15a-h include: new FRP patches (not retired) 1504 for strengthening beam corners; 1505: Glue used to join components, including boards 101, which are glued together; 902: Protruding bear claw screws as shown in Fig. 9; 702: chunks of retired FRP glued in place; 1507: Arrows indicating how the beam should be temporary pressed (clamping) for improved glue strength if screws are not used; 1508: Large arrow showing the direction in which the beam should be placed on concrete plate 1501; 101: Retired FRP boards, 10 mm thick, approximately 100 mm wide, and several meters long; 903: Protruding bear claw screws, serving a dual role of clamping glued board 101 and transmitting forces from the concrete plate; 1506 is the board 101 combined with cured concrete plate 1502. 703: Small 10 mm diameter shallow holes for strengthening the bond between concrete and the beam with a 1 mm diameter through hole (not visible) for air escape during concrete filling; 1511: double side reinforcement made of flat boards; 1509: End of a wind turbine blade cut out, suggesting minimal effort and strong beam/girder use instead of 1511; 1510: Element from a wind turbine blade, ready to be cut out for strong beam/girder reinforcement instead of 1511; U-shaped board101 from a wind turbine blade, provides another example of existing components used after cutting out, with minimal effort for use instead of FRP element shown in Fig. 15b; 1512 is an I-beam made of boards 101; 1513 is a middle part of untypical I-beam, which has slightly arc bottom; 602 is internally reinforced concrete similar to fig.6a-c.

The procedure for preparing element shown in Fig. 15a is similar to that depicted in Fig. 6a-c and involving the gluing of the FRP patches 1504 and protruding elements, as well as making holes. The ready assembled unit shown in Fig. 15a is then placed into fresh, soft concrete, where tensile forces similar to those in Figs. 11a-b can be applied to board 1506 if need occurs. The concrete is vibrated, and then allowed to cure. Element shown in Fig. 15c is analogous to elements shown in Fig. 15a and 15b, showcasing alternative shapes achievable with retired FRP reinforcement.

It's noted that the bottom of element shown in **Fig. 15c** demonstrates the use of pre-existing shapes cut from windmill blades and other retired FRP materials to optimize costs, achieving units similar to triangles based on 1511 but using end of a retired wind turbine blade cut out 1509 for narrow triangles or element from a wind turbine blade, ready to be cut out element 1510 for wider, stronger triangles. Element shown in Fig. 15d presents another efficient beam/girder type, utilizing U-shaped board 101 from a wind turbine blade, a nearly half-circle cut from retired windmill blades.

**Fig. 15e** shows how to make an I-beam from retired FRP, as representative of many known beams types. Prepare four clean boards 101 as shown (dimensions can be changed here in e.g. height 300mm, thickness 20 mm, and 4m long) apply glue 1505 and clamp with temporary force (as arrows depict) until glue cures. Than the surface which will be in contact with concrete can be modified as disclosed in this application for better bonding, this is not shown. Protect the surfaces with anti-moisture paint. When paint cures I-beam is ready to be glued (and screwed if need exists) to existing, cured flat concrete or to be submerged in fresh concrete as in fig. 15g or poured concrete on it or placed on fresh concrete similar to fig.15a so the effect shown at fig. 15f is similar to fig. 15b. Fig. 15h shows side view of untypical I-beam, it is made of 3 elements and middle board 1513 differs from the middle board 101 at fig. 15e because 1513 has bottom edge cut as part of circle, the right and left side of 1513 has height 250 mm and height in the middle of 1513 is 350 mm. So the bottom board 101 glued to 1513 is slightly bended. Fig. 15h shows example of shape not possible to produce by technology of pultrusion or extrusion type, but with retired FRP elements it is easy to make bending of one or more of the elements if there is need for such bending. Fig. 15i depicts the U-shaped board 101 as in the case of fig. 15d but the edges of the board 101 are simply placed in fresh concrete. What is not shown is that the surface of the U-shaped board101 connecting with concrete should be modified in ways depicted in this application for better bonding with concrete. Fig. 15i shows the board 101 after concrete is cured and it is shown with concrete plate 1502 up, similar to fig. 15b.

**Figures 16a-c** show three types of dowel bars reinforcement made of retired FRP. Fig. 16a (upper) shows a retired FRP dowel bars 1602, 1603, 1604 having different cross-sectional shapes (rectangular, oval, and circular) with a length of 300-700 mm, a height of 40 mm and a width (radius for round) of 20 mm. They can be done by pre-cutting the board 101 with a saw and fine machining the long rectangle with CNC and/or lathe and/or sandpaper. When the desired shape has been achieved, it is best to paint it with a coating of 1601, i.e. a 1 mm layer of a bond-breaking substance (like *'Tectyl 605' or other* Dowel Bar De-Bonding Paint). All side views do not show a layer of 1601, which should be added as the outside layer for better performance as dowel bar.

**Fig. 16b** discloses a composite dowel bar, where 101 are the left and the right part made of retired FRP. Transmitting concrete 1605 is a compressive force transfer concrete (10 mm wide) like polymer concrete, polyester resin concrete (PRC), ultra-high-performance concrete or just strong concrete.

To prepare the component shown in Fig. 16b, use 2 boards 101 10 mm thick, 40 mm high and 300-700 mm long, then make shallow holes 703 in each 101 of the inner side, drill holes and glue in them round pegs 1008 and/or rectangular pegs 1607 leaving a distance of 10 mm between both 101 to place fresh transmitting concrete 1605. Cover with temporary tape and pour transmitting concrete 1605, vibrate and wait for transmitting concrete 1605 to cure. Inspect and paint around with coating 1601.

To make the component shown in Fig. 16c follow the procedure in Fig. 16b until the both boards 101 are ready. Cut shallow grooves 3 mm deep and 3 mm wide in each inner side of the boards 101using a buzz saw or CNC. Drill two holes and glue in them round pegs 1008 as spacers, leaving 10 mm space for the transmitting concrete 1605. As before tape it around with tape and pour fresh transmitting concrete 1605 between both boards 101, vibrate and wait for it to cure. The joined boards 101, and the middle transmitting concrete 1605 is the composite Dowel Bar to be coated with 1 mm bond breaking substance 1601. One can use preferably silicon or rubber based moulds instead of tape for mass production of fig.16b-c Dowel Bars. One may consider prestressing those bars similar to examples from fig.11a-b.

**Figures 17a****-c** show preparing a construction reinforcement using effective cuts of retired windblade. Some FRP windlbades are made with a stronger "box" inside the aerofoil profile depicted at fig. 17a with wide black trapezoid box. These several meters long "T"-shaped boards 101 can be obtained with only 3 cuts - where the point of cut is marked with buzz saw symbol and dashed line (cutting). Figure 17a shows also elements, which are other several meters long "T"-shaped boards 101 obtainable with only 3 cuts. In fig.17b the joint of T-shaped boards 101, glued and screwed together, is strengthened using additional boards 101. The object in fig. 17b is an example of cross-section of several meters long reinforcement (holes 104 are not shown) which can be placed inside a concrete vertical pillar or to be joined with similar structures to create even larger reinforcement. The element in Fig. 17b has the advantage of a small cut and little effort but large reinforcement. There are not shown ways of improving bonding with concrete, those disclosed in this document should be considered.

**Fig. 17c** shows also effective large reinforcement using the existing FRP "box" of a retired FRP windblade. With a few additional retired FRP boards 101, a strong reinforcement is created that can become the sole reinforcement or can be combined with other similar structures if even larger reinforcement is needed.

**Figures 18a, 18b****, and** **18c** disclose the procedure of making holes and convex elements for strengthening bond between FRP and concrete. The advantage of this process is not adding additional elements. 101 - retired FRP plate 10 mm thick; 1801 - chisel like tool, manual or robotised to leverage upper layer of the rectangle; 1802 - cuts 5 mm deep in 101 done with cutting tool/process like saw, buzzsaw, plasma cutter, laser cutter, water cutter, milling, etc. Procedure shown in Fig. 18a involves making cuts half the thickness of FRP, 3 cuts of a rectangular, one of them is far wider - 3 mm (two others less than 1mm). The missing fourth side of the rectangle will be made by braking the leveraged piece. Use a chisel like tool to leverage up upper layer of the rectangle as shown by the arrows. After making the rectangular convex piece, apply polymer for water resistance and strengthening the convex element. Fig. 18b shows a process similar to Fig. 18a, leveraging the triangle piece from two sides. Rest of the process is the same as on Fig. 18a. This examples shown at figures 18a and 18b are to show how different geometrical shapes can be made from FRP to make hole and convex piece at one process. Fig. 18c shows process similar to Fig.18a and 18b, but no cuts are made, Step 1: drill the hole 1805 with shallow angle like 15 degrees to FRP level to drill half of the width of the FRP board 101. The hole can be made by drilling 1803. Step 2, the force shown by the arrows using a strong bar 1804 is applied to break "the ceiling of the hole 1805" to make the convex element 1806. Step 3 (Fig. 18c) includes applying the epoxy 1005 to provide water resistance and reinforce the convex element 1806.

**Figure 19** shows a process of cutting of retired wind blade and other retired FRP elements. It employs measuring devices 1901 like scanners (laser, visual, ultrasound, lidars and others) moving on drones, or otherwise or static, Roentgen scanners to picture inside inhomogeneities or similar equipment. The connection 1902 by wire, optical cable or wireless is capable of transmitting information from the measuring device 1901. The control unit 1903 may be a computer or similar hardware with software capable of reading information received through the connection 1902 from the measuring device 1901 and calculating (on site or via other connected computers) how to cut the windmill blade or other retired FRP elements. The figure shows also a cable or wireless connection 1904 transmitting signals/information from the control unit 1903 to the carriage 1907 and a cable or wireless connection 1905 transmitting signals/information from the unit 1903 to the cutter 1906. The cutter 1906 can be a band saw, buzzsaw, rotary saw, plasma cutter, waterjet, jet powder cutter, electron beam cutter, CNC, chemical cutter, other mechanical cutter, laser cutter, etc. It can be controlled by a 1903.

Preferably the construction comprises an upper and a lower boards 101, two side boards 101 and means for stabilizing the folded construction in a 90 degrees angle position, and means for allowing the construction to be folded and unfolded. The means for stabilizing the folded construction are selected from the group comprising strings 2001, 2003, triangular elements 2005, 2007, squared sticks 2026, bear claw screws 2006, and/or combination of them and the means for allowing the construction to be folded and unfolded are selected from the group comprising hinges 2002, 2012, plugs 2014, screws 2018, wedges 2019, strings 1306, ropes 1103, boards 1106, 1107 and/or combination of them.

**Figures 20a****-f** disclose folding structures made from retired FRP for reinforcement of concrete.

**Fig. 20a** shows flat, an unfolded structure 2008 on the left and in folded state on the right. It consist of the upper and the lower boards 101, two side boards 101 made from retired FRP, two not flexible strings 2001 and two flexible strings 2003. Four hinges 2002 might be traditional hinges or preferably living hinges from new or retired flat pieces of polymers easy to glue to FRP boards. Hinges 2002 can be even made from strong duct tape. Hinges allow movement of the boards 101, while not flexible strings 2001 restrict movement of FRP boards to 90 degrees angle position. Flexible strings 2003 (rubber kind or long springs) with hook each at the end which is not glued to 101 is to make constant tension against the restricting strings 2001. Each hook is to be hooked at its respective hole in 101, hooks and respective openings are not shown.

Side boards 101 are 20mm thick and 700 mm wide and about 2 meters long. Each board should have 100 mm diameter through holes (not shown), for easy flow of fresh concrete, evacuation of air and strong bonding between reinforcement and the concrete. Other means for improving such bonding disclosed in this document might be of use.

Hinges 2002 are also 2 m long. Length of each string 2001 and 2003 should be made such, that after folding, the structure has a rectangular cross-section, as in Fig. 20a.

To make the structure 2008, prepare boards 101, drill holes 104 and attach hinges 2002. Glue in restricting strings 2001 and one end of each flexible strings 2003. Attach hook on the other end of each 2003 and make hole for each hook. Inspect the structure and protect against moisture with paint.

After transporting the structure 2008 in flat state fold it up and hook hooks into their holes. Place the folded structure 2008 into desired space and secure to the ground, pour fresh concrete into it and on it.

**Fig. 20b** shows a structure 2009 similar to the structure 2008 at fig. 20a, but instead of strings, small triangular elements of FRP 2005 and 2007 are used to stabilize the folded structure 2009 before pouring concrete. There are two triangle shaped pieces 2005 which are installed on hinge 2002. The triangular element 2007 is not hinged but can rotate on axle 2004. Each triangular element 2005 and 2007 has a bear claw screw 2006 (or genuine screw which head is protruding 5mm). There is also a carved groove (not shown) for each 2006 to lock the whole structure 2009 stable.

To produce the structure 2009 follow the procedure according to the structure 2008, but instead of strings 2001 and 2003 attach triangular elements 2005 and 2007 with their screws 2006 . Make groves in upper and lower boards 101 according to movement of each triangular element 2007 with locking ending in the groove. Following examples at fig. 20a-b one can make snap-fit locking for structure as added (glued) snap-fit elements or snap-fit cut in retired RFP elements as shown at fig. 20e.

**Fig.20c** shows 3-element folding structure 2016 where hinges 2012 and 2013 are shown in detail. They are thin (less than 1 mm) pieces of easy to glue polymer which is flexible to bend like polyethylene or polycarbonate sheets, preferably retired.

The hinge 2012 has a rectangular shape with a width of 400 mm and a length of 2 m, while the hinge 2013 has also a rectangular shape with a width of 400 mm but a length of 1 m with one corner cut out as shown in fig. 20c. The triangular element 2011 is a right-angled triangle with one side 1020 mm long and the other 1000 mm long, the width is as the board 101 -20 mm.

On the side of the lower board 101 two plugs 2014 with a diameter of 5 mm protruding 10 mm are installed, which will fit tightly into the two holes 2015 in the triangular element 2011 when the structure is folded. Plugs 2014 with their holes 2015 will make a stable structure 2016 for concrete pouring. The element 2010 is a snap-fit mechanism as an alternative to the plugs 2014 and holes 2015 as a locking mechanism of the structure 2016.

**Fig. 20d** shows folding a structure 2020. It consists of 4 boards 101 made of retired FRP with overlapping "tooth" edges, 3 "teeth" on each edge. Each element has 100 mm diameter through holes 104 drilled for improved concrete pouring and bonding to cured concrete. Other means of improving bonding from this application should also be considered.

Outside dimensions of two depicted in Fig. 20d boards 101 are 300 mm wide, 500 mm long and 20 mm thick. Top and bottom boards 101 are 500 mm wide, 500 mm long and 20 mm thick. The length can be several meters for longer reinforcements.

There are three metal axes 2017, with a diameter of 3 mm between the boards 101, which allow the structure 2020 to be folded easily. The connection between the external boards 101 should be secured with screw 2018 with or without glue. Other screw can be used to secure the folded structure 2020 and/or the wedge 2019 to be hammered in between teeth. As before, after transporting 2020 in the unfolded state, fold it up and secure with wedges/nails/screws/glue. Place folded 2020 into desired space and secure it to the ground (or supports), pour fresh concrete into it and on it. Folded 2020 may also work as beam/girder reinforcement.

**Fig. 20e** shows the alternative to the axial connection in the structure 2020, the ends of the 'teeth' of the boards 101 are machined so that one board 101 can be pushed into another board 101 of the structure, while the snap-fit mechanism 2021 locks both boards 101 in place, when they are perpendicular as shown. The snap-fit mechanism 2021 is presented on the right, it is a narrow, flexible part which springs into its place when the boards 101 are perpendicular to each other, locking them in place.

**Fig.20f** depicts a folding reinforcement structure 2025 with a triangular cross-section made of a base FRP board 101 and two FRP boards 101 being folding up arms of the triangle. They are connected with grooves and protruding shapes and also are taped with duct tape as hinges 2022, internal hinges 2023 and external hinge 2024.

To prepare the structure 2025 use flat retired FRP 0,5 m wide, 2 m long and 20 mm thick. Make two 4 mm (wide and high) grooves 5 mm from the edges as shown, obtaining a base FRP board 101. Other boards 101 are also 2 m long and 20 mm thick but 400 mm wide. Machine 4 mm grooves and 3 mm protruding shapes also 5 mm from its edge as shown on fig. 20e. Consider drilling holes as on fig. 20d and other disclosed solutions for better bonding to concrete. Paint with anti-moisture paint and stick three 2 m long duct tape 40 mm wide as the hinges 2022, 2023, and 2024. As before after transporting 2025 in flat state, fold it up in desired space and secure it to the ground, pour fresh concrete into it and on it.

**Fig. 20g** is an another embodiment of the structure 2008 from fig. 20a. Instead of strings, a squared FRP stick 2026 is used to stabilize a folded structure 2027.

To make the structure 2027 follow the procedure for the structure 2008 but don't use strings 2001 and 2003 as well as hooks and openings for them. Instead cut a square stick 2026 from retired FRP with width of 20 mm and length 1200 mm. Cut two incisions in it, 22 mm wide, 13 mm deep, 10 mm from each end, and angled 45 degrees, as shown in the figure 20g,. If necessary, make a second square stick 2026 for the other end of the structure 2027. The squared stick 2026 should be attached to unfolded side boards 101 with paper tape or similar easy to break temporary fastening element. Painting with anti-moisture paint will add longevity of this reinforcement. Holes and incisions in boards 101 should be considered for better bonding with concrete.

As before after transporting the structure 2026 in unfolded state, fold it up in desired space and use the square stick 2026 to make it straight, self-standing. Secure it to the ground, pour fresh concrete into it and on it.

Yet another aspect of the invention is a use of the construction element defined above in the construction of roads and load-bearing structural elements like foundations, ceilings, footings, girders, columns, stairs, beams, retaining walls, concrete slabs. **Fig. 21** is an example of a ground compressing equipment 2105 made of a large retired FRP board 101 with a concrete arch 2101 and several strong ropes 2102 (steel with corrosion protection, polymer or other) . Also important is a fabric or a similar filter material 2104 that retains solid particles but allows fluid (water) to pass through. The ropes 2102 are in constant tension to compress ground, the board 101 comprises a number of tiny holes that allow water, but not solid particles, to passthrough. If there is no solid wall on the other side, then the compressing equipment 2105 can be reflected opposite to the first compressing equipment 2105. The whole equipment shown in fig.21 can significantly strengthen ground without need of removing the ground, both ground compressing equipment 2105 and tensioned ropes stay in ground.

To prepare the compression equipment 2105 first a large flat board 101 of retired FRP for example 9 m long, 3 m high and minimum 10 mm thick should be prepared. Prepare the board 101 for concrete by drilling fifty 30 mm diameter holes (not on picture) and other ways disclosed in this application to make the bonding with concrete strong. Drill approximately one thousand through holes in the board 101 with a diameter of 1 mm or slightly larger if anti-moisture solution will be used. Position the concrete arch as shown in fig 21, the dimensions to be determined according to the expected forces. Make through holes for ropes in the concrete and in the board 101. When concrete cures, glue the filtering material 2104 to the board 101 with a small amount of adhesive spots to allow water to flow through. At the selected site dig two parallel trenches 9.5 m long, 3 m deep (or deeper if the unit is to compress deeper ground) and approximately 2 m wide (depending on the arch). Install both compressing equipment 2105 in the trenches as shown in figure. Dig narrow perpendicular paths for cables/ropes and install ropes 2102. Use some additional filtering material 2104 around the ropes. Pull each rope 2102 to the desired tension, use steel or retired FRP or other polymer elements 2103 with hole to secure the concrete and cable connection and secure it so that the tension remains long (for example with a threaded connector). Prepare water escape ways from the outside of each 2105. Use ground or gravel to fill holes, paths and trenches in the ground, check and correct tension if necessary. Instead of digging perpendicular open paths for the ropes one can drill or push holes into the ground for the ropes 2102.

## Claims

1. A construction reinforcement suitable for use in concrete-based systems, comprising at least one board (101) made of Fiber Reinforced Polymers (FRP), **characterized in that** the board is made of retired FRP, and wherein the construction reinforcement comprises means for improving adhesion to concrete and the force transmission.

2. The construction reinforcement according to claim 1, **characterized in that** the means for improving adhesion to concrete and the force transmission are selected from the group comprising protruding elements (103), through holes (104, 110), grooves (315, 703), indentations (701), adhered loose materials and/or combination thereof.

3. The construction reinforcement according to claim 2, **characterized in that** the protruding elements (103) are selected from the group comprising screws (106, 902, 903), pegs (108, 1004, 1403, 1404, 1607), bolts (1001, 1002, 1003), dowels, plugs (2014), expansion anchors, fasteners made of retired FRP (102, 504), strings (301, 313, 1103, 1401), strands, knots (1402), retired fishing nets (302), bottle cups (303), polymer tines (307), rebars (322), FRP chunks (702), convex elements (1008, 1806), polymer elements, nails and/or combination thereof.

4. The construction reinforcement according to claim 2, **characterized in that** the adhered loose materials ale selected from the group comprising sand (308), polymer elements, FRP elements, ground FRP dust, epoxy resin (310), gravel, aggregates, quartz, broken glass, perlite, ceramic, corundum, polyurethane powder, pumice, silicon carbide, and/or combination thereof

5. The construction reinforcement according to claim 2, **characterized in that** the through holes (104) have dimensions in the range from 10 to 990 mm, wherein the drilling angle is in the range from 40 to 140 degrees.

6. The construction reinforcement according to any of claims 1-5, **characterized in that** the board (101) is substantially flat or is profiled into a shape selected from a group comprising a comb, an angled board, a U-shaped board, a L-shaped board, H-shaped board, T-shaped board and/or a circular board.

7. The construction reinforcement according to any of claims 1 to 6, **characterized in that**, the boards (101) are butt jointed or at least partially overlapping.

8. The construction reinforcement according to claim 7, **characterized in that**, the butt joint is a straight joint, a diagonal joint, a structural diagonal joint (1006), a multiple tongue and groove joint (1007) or a structural joint (1008).

9. The construction reinforcement according to claim 7, **characterized in that** the boards (101) are jointed by adhesive and/or by other means, selected from the group comprising dovetail, pegs (108, 1004, 1403, 1404), dowels, plugs (2014), expansion anchors, bolts (1001, 1002, 1003), ultrasound welding, nails, screws (106, 902, 903), and/or combination thereof.

10. The construction reinforcement according to any one of claims 1 to 9, **characterized in that** the boards (101) are arranged in at least two parallel planes connected by FRP brackets (601), wherein the axial distance of the planes is in the range from 20 mm to 990 mm.

11. The construction reinforcement according to claims 1 to 5, **characterized in that** the construction comprises an upper and a lower boards (101), two side boards (101) and means for stabilizing the folded construction in a 90 degrees angle position, and means for allowing the construction to be folded and unfolded.

12. The construction reinforcement according to claim 11, **characterized in that**, the means for stabilizing the folded construction are selected from the group comprising tape, strings (2001, 2003), triangular elements (326, 2005, 2007), squared sticks (2026), bear claw screws (2006), and/or combination of them and the means for allowing the construction to be folded and unfolded are selected from the group comprising hinges (2002, 2012), plugs (2014), nails, screws (2018), wedges (2019), elastic strings (1306), comb elements (1309), 3D printed elements (1308), strings (1306), ropes (1103), boards (1106, 1107), elements with snap-fits (324) and/or combination thereof.

13. A construction element comprising the construction reinforcement specified in claims 1-12 embedded in concrete of the thickness in the range from 20 mm to 9900 mm, wherein the concrete comprises aggregates, water and cement, and wherein the cement is selected from the group comprising Portland cement, geopolimers, fly ashes, blast furnace slag, belite cement, cement from agricultural ashes, aluminous cement, pozzolanic cement, silica fume, polymer functioning as binder, metakaolin, and and/or any combination thereof.

14. A method for obtaining the construction element specified in claim 13, comprising following steps:
a) placing in the board (101) the means for improving adhesion to concrete and force transmission, selected from the group comprising: screws (106, 902, 903), pegs (108, 1004, 1403, 1404), bolts (1001, 1002, 1003), dowels, plugs (2014), expansion anchors, fasteners made of retired FRP (102,504), strings (301, 313, 1103, 1401), strands, knots (1402), retired fishing nets (302), bottle cups (303), polymer tines (307), rebars (322), FRP chunks (702), convex elements (1008, 1607, 1806), grooves (315, 703), indentations (701), adhered loose materials selected from the group comprising sand (308), polymer elements, FRP elements, ground FRP dust, epoxy resin (310), gravel, aggregates, quartz, broken glass, perlite, ceramic, corundum, polyurethane powder, pumice, silicon carbide, and/or combination thereof **AND/OR** drilling the through holes (104, 110) in the boards (101), in the distance not less than 10 mm from the edges of the board (101) and from any other hole (104, 110);
b) optionally, covering all uncoated cut edges of the board (101) with polymer;
c) jointing of boards (101);
d) pouring the reinforcement construction obtained in steps a)-c) with concrete material with a thickness of at least 20 mm or dipping the reinforcement construction into fresh concrete material with a thickness of at least 40 mm;
e) optionally vibrating and curing the concrete at a time of at least 2 hours.

15. The method according to claim 14, **characterized in that**, after step c) protruding elements (103) on the joints between boards (101) using adhesive and/or other means, selected from the group comprising nails, screws (106, 902, 903), pegs (108, 1004, 1403, 1404), bolts (1001, 1002, 1003), dowels, plugs (2014), expansion anchors, fasteners made of retired FRP (102, 504), strings (301, 313, 1103, 1401), strands, knots (1402), retired fishing nets (302), bottle cups (303), polymer tines (307), rebars (322), FRP chunks (702), convex elements (1008, 1607, 1806), and/or combination thereof are installed.

16. The method according to claim 14, **characterized in that** the polymer is selected from the group comprising gelcoat, epoxy resin, polyurethane coatings, phenolic coatings, urea-formaldehyde coatings, polyester coatings, vinyl ester resins, silicone coatings, acrylic coatings, alkyd coatings, nitrocellulose coatings, melamine-alkyd coatings, nanocoatings and/or any combination thereof.

17. The method according to claim 14, **characterized in that** before pouring the concrete in step d) the reinforcement construction is prestressed by pulling a tensile force from 0,5 kN to 990 kN from both opposite ends of the construction.

18. The method according to claim 15, **characterized in that**, the adhesive is selected from the group comprising polyurethane adhesives (PUR), epoxy adhesives, cyanoacrylate adhesives, acrylic adhesives, silicone adhesives, construction adhesives, contact adhesives, hybrid adhesives, cementitious adhesives, and/or parquet adhesives.

19. A use of the construction element specified in claim 13 in the construction of roads and load-bearing structural elements like foundations, ceilings, footings, girders, columns, stairs, beams, retaining walls, bridges, concrete slabs, prefabricated concrete modules.

## Amended claims

### Amended claims in accordance with Rule 137(2) EPC.

1. A construction element suitable for use in concrete-based systems comprising a construction reinforcement,
wherein a construction reinforcement, comprising boards (101) made of Fiber Reinforced Polymers (FRP), **characterized in that** the boards are made of recycled FRP, the boards (101) are butt jointed or at least partially overlapping, and wherein the construction reinforcement comprises means for improving adhesion to concrete and the force transmission
**characterized in that** a construction reinforcement is embedded in concrete of the thickness in the range from 20 mm to 9900 mm, wherein the concrete comprises aggregates, water and cement, and wherein the cement is selected from the group comprising Portland cement, geopolimers, fly ashes, blast furnace slag, belite cement, cement from agricultural ashes, aluminous cement, pozzolanic cement, silica fume, polymer functioning as binder, metakaolin, and and/or any combination thereof,

2. The construction element according to claim 1, **characterized in that** the means for improving adhesion to concrete and the force transmission are the protruding elements (103) selected from the group comprising screws (106, 902, 903), pegs (108, 1004, 1403, 1404, 1607), bolts (1001, 1002, 1003), dowels, plugs (2014), expansion anchors, fasteners made of retired FRP (102, 504), strings (301, 313, 1103, 1401), strands, knots (1402), retired fishing nets (302), bottle cups (303), polymer tines (307), rebars (322), FRP chunks (702), convex elements (1008, 1806), polymer elements, nails and/or combination thereof.

3. The construction element according to claim 1, **characterized in that** the means for improving adhesion to concrete and the force transmission are the adhered loose materials selected from the group comprising sand (308), polymer elements, FRP elements, ground FRP dust, epoxy resin (310), gravel, aggregates, quartz, broken glass, perlite, ceramic, corundum, polyurethane powder, pumice, silicon carbide, and/or combination thereof

4. The construction element according to claim 1, **characterized in that** the means for improving adhesion to concrete and the force transmission are the through holes (104) having dimensions in the range from 10 to 990 mm, wherein the drilling angle is in the range from 40 to 140 degrees.

5. The construction element according to any of claims 1-4, **characterized in that** the boards (101) are substantially flat or profiled into a shape selected from a group comprising a comb, an angled board, a U-shaped board, a L-shaped board, H-shaped board, T-shaped board and/or a circular board.

6. The construction element according to any of claims claims 1-5, **characterized in that**, the butt joint is a straight joint, a diagonal joint, a structural diagonal joint (1006), a multiple tongue and groove joint (1007) or a structural joint (1008).

7. The construction element according to any of claims claims 1-6, **characterized in that** the boards (101) are jointed by adhesive and/or by other means, selected from the group comprising dovetail, pegs (108, 1004, 1403, 1404), dowels, plugs (2014), expansion anchors, bolts (1001, 1002, 1003), ultrasound welding, nails, screws (106, 902, 903), and/or combination thereof.

8. The construction element according to any one of claims 1 to 7, **characterized in that** the boards (101) are arranged in at least two parallel planes connected by FRP brackets (601), wherein the axial distance of the planes is in the range from 20 mm to 990 mm.

9. A method for obtaining the construction element specified in claims 1-8, comprising following steps:
a) placing in the boards (101) the means for improving adhesion to concrete and force transmission, selected from the group comprising: screws (106, 902, 903), pegs (108, 1004, 1403, 1404), bolts (1001, 1002, 1003), dowels, plugs (2014), expansion anchors, fasteners made of retired FRP (102, 504), strings (301, 313, 1103, 1401), strands, knots (1402), recycled fishing nets (302), bottle cups (303), polymer tines (307), rebars (322), FRP chunks (702), convex elements (1008, 1607, 1806), grooves (315, 703), indentations (701), adhered loose materials selected from the group comprising sand (308), polymer elements, FRP elements, ground FRP dust, epoxy resin (310), gravel, aggregates, quartz, broken glass, perlite, ceramic, corundum, polyurethane powder, pumice, silicon carbide, and/or combination thereof **AND/OR** drilling the through holes (104, 110) in the boards (101), in the distance not less than 10 mm from the edges of the board (101) and from any other hole (104, 110);
b) optionally, covering all uncoated cut edges of the board (101) with polymer;
c) jointing of the boards (101);
d) embedding the reinforcement construction obtained in steps a)-c) in concrete material with a thickness of at least 20 mm to 9900 mm;
e) optionally vibrating and curing the concrete at a time of at least 2 hours.

10. The method according to claim 9, **characterized in that**, after step c) protruding elements (103) on the joints between boards (101) using adhesive and/or other means, selected from the group comprising nails, screws (106, 902, 903), pegs (108, 1004, 1403, 1404), bolts (1001, 1002, 1003), dowels, plugs (2014), expansion anchors, fasteners made of retired FRP (102, 504), strings (301, 313, 1103, 1401), strands, knots (1402), retired fishing nets (302), bottle cups (303), polymer tines (307), rebars (322), FRP chunks (702), convex elements (1008, 1607, 1806), and/or combination thereof are installed.

11. The method according to claim 9, **characterized in that** the polymer is selected from the group comprising gelcoat, epoxy resin, polyurethane coatings, phenolic coatings, ureaformaldehyde coatings, polyester coatings, vinyl ester resins, silicone coatings, acrylic coatings, alkyd coatings, nitrocellulose coatings, melamine-alkyd coatings, nanocoatings and/or any combination thereof.

12. The method according to claim 9, **characterized in that** before pouring the concrete in step d) the reinforcement construction is prestressed by pulling a tensile force from 0,5 kN to 990 kN from both opposite ends of the construction.

13. The method according to claim 10, **characterized in that**, the adhesive is selected from the group comprising polyurethane adhesives (PUR), epoxy adhesives, cyanoacrylate adhesives, acrylic adhesives, silicone adhesives, construction adhesives, contact adhesives, hybrid adhesives, cementitious adhesives, and/or parquet adhesives.

14. A use of the construction element specified in claims 1-8 in the construction of roads and load-bearing structural elements like foundations, ceilings, footings, girders, columns, stairs, beams, retaining walls, bridges, concrete slabs, prefabricated concrete modules.
